

Patented Nov. 4, 1924.

## UNITED STATES PATENT OFFICE.

COLIN G. FINK, OF YONKERS, NEW YORK, ASSIGNOR TO CHILE EXPLORATION COMPANY, OF NEW YORK, N. Y., A CORPORATION OF NEW JERSEY.

## ALLOY.

No Drawing.

Application filed January 26, 1921. Serial No. 440,167.

*To all whom it may concern:*

Be it known that I, COLIN G. FINK, a citizen of the United States, residing at Yonkers, in the county of Westchester, State of New York, have invented certain new and useful Improvements in Alloys; and I do hereby declare the following to be a full, clear, and exact description of the invention, such as will enable others skilled in the art to which it appertains to make and use the same.

This invention relates to alloys and has for its object the provision of an improved alloy adapted particularly for withstanding attacks from corrosive liquors.

Metallic receptacles generally are not adapted for the handling of corrosive liquids because of the corroding or disintegrating effect which such liquids have upon the metal. Alloys of various composition have heretofore been proposed for resisting the corrosive action of particular liquors. The present invention contemplates the provision of an improved alloy which is especially resistant to the corrosive action of acid liquors and more particularly sulfuric acid liquors containing appreciable amounts of nitrates and chlorides.

The improved alloy of the invention is made up principally of cobalt and silicon. In its preferred form, the alloy also contains manganese and chromium, together with a certain amount of carbon. I have found an alloy of the following composition to possess very excellent corrosive resisting properties: 11-13% silicon, 4-6% chromium, 4-6% manganese, 0.8-1.2% carbon, and the balance cobalt. The foregoing proportions may be varied in about the following percentages without material alteration of the desirable properties of this preferred form of the invention: silicon, 10-15%, manganese 2-8%, chromium 2-12%.

In its preferred form, the principal constituent of the alloy of the invention is cobalt. However, I have found that the cobalt may be replaced to a certain extent by manganese or chromium, or even by a small percentage of nickel, although the substitution of nickel for part of the cobalt is not recommended except where the cost of the alloy is an important factor, because nickel-silicon alloys are far less corrosive-resisting than cobalt-silicon alloys. Accordingly, if desired, 5 to 30 parts (per 100 parts) of the

cobalt content of the alloy may be replaced by manganese, or 5 to 12 parts (per 100 parts) of the cobalt content may be replaced by chromium, or 5 to 8 parts (per 100 parts) of the cobalt content may be replaced by 60 nickel, without objectionably altering the advantageous properties of the alloy as a corrosion-resisting material.

As a result of my investigations and researches, I have found that an improved alloy resistant to corrosion from acid liquors, and in particular sulfuric acid liquors containing chlorides and nitrates, can be produced from cobalt and silicon, by combining these metals in the form of a cobalt-silicon 70 alloy of appropriate composition. I have also found that when cobalt and silicon are appropriately alloyed together with a small amount of manganese and carbon, the resulting alloy has greater strength and pos- 75 sseses other desirable qualities which adapt it particularly for use in the manufacture of corrosion-resisting receptacles, pipes, etc. I have, moreover, found that the addition of chromium, or other equivalent metal of the 80 chromium group, such as tungsten, molybdenum or uranium, to the cobalt-silicon alloy imparts thereto further advantageous characteristics.

I have found that commercial cobalt is 85 well adapted for use in the production of alloys in accordance with the principles of the present invention. Cobalt has a marked affinity for carbon and, if desired, may be preliminarily combined with the amount of 90 carbon to be incorporated in the alloy. The proportion of carbon, of manganese, of chromium, and of silicon can be somewhat varied, but in general neither the carbon, the manganese, the chromium or chromium 95 group metal, nor the silicon should be too low, since if these metals are not present in sufficiently large amounts the resulting alloy will not possess the desired corrosion-resisting properties. On the other hand, the 100 carbon, the manganese, the chromium and the silicon content should not be too high. A high silicon content results in a decrease in the strength of the alloy and also increases the tendency of the alloy to corrode. If the carbon content is too high, the carbon separates out in a graphitic form. I have obtained the best results with a carbon content slightly in excess of the amount 105 which can be combined, so that there is a 110

small amount of fine graphitic carbon, such as will give a grey surface to the fracture, but without any large excess of graphitic carbon.

5 I have found that the alloys of cobalt and silicon are distinguished from alloys of other more or less similar metals with silicon in their availability for use as corrosion resisting materials. The advantageous properties of the cobalt-silicon alloys are due, I believe, to the peculiar characteristics of these alloys. Microphotographs of cobalt-silicon alloys containing about 12 to 15% of silicon indicate that the silicon is in part 10 present as such or as cobalt-silicide ( $Co_2Si$ ) in solid solution in the cobalt, while a large part is present in the form of a eutectic made up of a mixture of cobalt silicide ( $Co_2Si$ ) in the cobalt. The microphotographs 15 indicate that the resistance to corrosion may be largely due to the presence of the silicon and of the cobalt silicide.

I have found that a maximum strength against flexure is obtained when the silicon 20 content of the cobalt-silicon alloy is about 12-15%. For example, a flexure strength of around 6200 pounds per square inch (unit beam 1 inch square 12 inch span) has been possessed by alloys of this silicon content. 25 Both any material increase and any material decrease in the silicon content of the alloy seem to decrease the mechanical strength of the alloy, and, in general, the greatest strength is obtained at between 12 and 15% 30 of silicon. In its breaking strength, the improved alloy of the invention is to be distinguished from an alloy of iron and silicon, where, for example, a similar content of silicon gives an alloy with a flexure strength 35 of about 1000 to 1500 pounds per square inch.

I have obtained good results with a carbon content of about 1% or between 0.5% and 40 1.2%, and with a silicon content of from 45 12 to 15%. Graphitic carbon, as hereinbefore pointed out, is objectionable beyond a certain small amount, but inasmuch as cobalt will combine more readily than iron with a small amount of carbon, it is possible 50 to include such a larger amount in the alloy without an objectionable amount of graphitic carbon being present.

The proportions hereinbefore mentioned 55 of the various ingredients of my improved alloy generally represent what I now believe to be the preferred form of the invention. However, I wish it to be understood that these specific proportions mentioned may be somewhat varied without departing from 60 the spirit of the invention. Thus, for example, I have found that by increasing the silicon content up to about 20%, I can bring the manganese content as high as 45%. This 65 is of particular advantage in that it tends to lower the cost of the alloy. In general, I

may say that an alloy embodying the principles of the invention in their complete aspect should contain from about 10 to 20% silicon, from about 2 to 45% manganese, from about 2 to 12% chromium or the 70 equivalent amount of tungsten, molybdenum or uranium, and the balance cobalt (including the aforementioned relatively small percentage of carbon). Moreover, it is to be understood that while certain advantages of 75 the invention are obtained without the inclusion of either manganese or a chromium group metal in the alloy that the presence of both of these metals is desirable, since their inclusion imparts to the alloy further 80 desirable properties. Small percentages (up to about 4%) of iron, titanium, aluminum, antimony, bismuth, or tin, may be present in the alloy without objectionable impairing its corrosion resisting properties. 85

In the production of the improved alloy of the present invention, I may employ cobalt with its normal impurities, including some small percentage of nickel, iron, manganese and carbon. I have obtained good 90 results with cobalt-containing around 4 to 7% of nickel and iron together. In the production of the alloy, I may proceed by melting the cobalt and adding charcoal thereto to increase its carbon content, or by simultaneously reducing a mixed oxide of cobalt, manganese and chromium (or other chromium group metal). I may then add the silicon together with the manganese to the molten cobalt, but I have found that the addition of the silicon to the cobalt results in a violent evolution of heat so that care should be taken to avoid the addition of such large amounts of silicon as will result 95 in objectionable overheating. The silicon can be added gradually or as carbide of silicon or it may be combined with a small amount of cobalt and the resulting alloy or mixture added to the remaining portion 100 of the cobalt. This violent evolution of heat which takes place when the silicon is added to cobalt is a further characteristic of the cobalt-silicon composition which distinguishes it from iron-silicon compositions. 105

I claim:—

1. An alloy containing cobalt in predominant amount, and more than 10 and up to 20% of silicon.
2. An alloy containing cobalt in predominant amount, 10 to 20% of silicon, more than 2 and up to 45% of manganese, and 2 to 12% of chromium.
3. An alloy containing cobalt in predominant amount, about 12 to 15% of silicon and about 2 to 8% of manganese.
4. An alloy containing cobalt in predominant amount, about 12 to 15% of silicon, and about 2 to 12% of chromium.
5. An alloy containing cobalt in predominant amount, about 12 to 15% of silicon,

about 2 to 8% of manganese, and about 2 to 12% of a chromium group metal.

6. An alloy containing cobalt in predominant amount, manganese from 2 to 45%, chromium from 2 to 12%, silicon from 10 to 20% and sufficient carbon to supply a small amount of graphitic carbon to the alloy.

7. An alloy containing cobalt in predominant amount, about 12 to 15% of silicon, about 2 to 8% of manganese and about 2 to 12% of a chromium group metal.

8. An alloy containing cobalt in predomi-

nant amount, 11 to 13% silicon, 4 to 6% chromium, and 4 to 6% manganese.

9. An alloy containing cobalt in predominant amount, 11 to 13% silicon, 4 to 6% of a chromium group metal, and 4 to 6% manganese.

10. An alloy containing cobalt in predominant amount, 11 to 13% silicon, 4 to 6% of a chromium group metal, 4 to 6% manganese, and 0.8 to 1.2% carbon.

In testimony whereof I affix my signature.  
COLIN G. FINK.